

# United States Patent [19]

Fadner et al.

[11] Patent Number: 4,537,127

[45] Date of Patent: Aug. 27, 1985

[54] **BLACK OXIDE LITHOGRAPHIC INK METERING ROLLER**

[75] Inventors: Thomas A. Fadner, LaGrange; Stanley H. Hycner, Bartlett, both of Ill.

[73] Assignee: Rockwell International Corporation, Pittsburgh, Pa.

[21] Appl. No.: 649,773

[22] Filed: Sep. 12, 1984

[51] Int. Cl.<sup>3</sup> ..... B41F 1/46; B41F 31/26

[52] U.S. Cl. ..... 101/141; 101/348; 101/451; 101/350; 29/132

[58] Field of Search ..... 101/141, 348, 349, 350, 101/451, 150, 170; 29/132

[56] References Cited

U.S. PATENT DOCUMENTS

2,530,282 11/1950 Brodie ..... 101/348 X  
2,578,921 12/1951 Cramer ..... 101/350  
3,613,578 10/1971 Heurich ..... 101/350

3,924,313 12/1975 Broderick ..... 101/350  
3,974,555 8/1976 Strohmeier ..... 29/132  
4,009,658 3/1977 Heurich ..... 101/348  
4,060,882 12/1977 Pospisil ..... 29/132  
4,287,827 9/1981 Warner ..... 101/148  
4,391,879 7/1983 Fabian ..... 29/132  
4,407,196 10/1983 Matalia ..... 101/229

FOREIGN PATENT DOCUMENTS

58-42463 3/1983 Japan ..... 101/350  
58-56855 4/1983 Japan ..... 101/348  
1585143 2/1981 United Kingdom ..... 101/349

Primary Examiner—Clyde I. Coughenour

Assistant Examiner—William L. Klima

[57] ABSTRACT

A steel ink metering roller for use in lithographic printing having an engraved surface that has been nitride hardened followed by an oxidizing process that results in a surface with a composition of mainly  $Fe_3O_4$ .

8 Claims, 9 Drawing Figures



Fig. 1.



Fig. 2.



Fig. 4.



Land Area  
44%

Fig. 3.



Fig. 5.



Fig. 6.



Fig. 7.



Fig. 8.



Fig. 9.



## BLACK OXIDE LITHOGRAPHIC INK METERING ROLLER

### BACKGROUND OF THE INVENTION

In the practice of conventional lithographic printing, it is essential to maintain sufficient water in the non-image areas of the printing plate to assure that image/non-image differentiation is maintained. That is, to assure that ink will transfer only to the image portions of the printing plate format. Many different dampening or water conveying systems have been devised and these systems can be referred to by consulting "An Engineering Analysis of the Lithographic Printing Process" published by J. MacPhee in the Graphic Arts Monthly, November, 1979, pages 666-668, 672-673. Neither the nature of the dampening system nor the nature of the dampening materials that are routinely used in the practice of high speed lithography are expected to place restrictions on the utilization of the improved metering roller of the present invention.

The dampening water in lithography is commonly supplied to the printing plate in the form of a dilute aqueous solution containing various proprietary combinations of buffering salts, gums, wetting agents, alcohols, fungicides and the like, which additives function to assist in the practical and efficient utilization of the various water supply and dampening systems combinations that are available for the practice of lithographic printing. Despite their very low concentrations, typically less than about one percent, the salts and wetting agents have been found in practice to be essential if the printing press system is to produce printed copies having clean, tint-free background and sharp, clean images, without having to pay undue and impractical amounts of attention to inking and dampening system controls during operation of the press. Apparently the dampening solution additives help to keep the printing plate non-image areas free of spurious specks or dots of ink that may be forced into those areas during printing.

It is well known in the art and practice of lithographic printing that ink is relatively easily lifted off, cleaned off, or debonded from most metallic surfaces, from most metal oxide surfaces and from virtually all high surface energy materials, such as the non-image areas of lithographic printing plates, by the action or in the presence of typical lithographic dampening solutions used in the printing industry. A similar phenomenon may occur when ordinary water or deionized water or distilled water is used without the dampening additives, but the debonding action of the water will be less efficient and will generally take place more slowly. In fact, lithographers have found that it is virtually impossible to produce acceptable lithographic printing quality efficiently or reproducibly using dampening water not containing the kinds of additives previously referred to.

Reference to R. W. Bassemir or to T. A. Fadner in "Colloids and Surfaces in Reprographic Technology", published by the American Chemical Society in 1982 as ACS Symposium Series 200, will relate that in the art of lithography the inks must be able to assimilate or acquire a quantity of water for the lithographic process to have practical operational latitude. Apparently the ink acts as a reservoir for spurious quantities of water that may appear in inked images areas of the plate, since water is continuously being forced onto and into the ink in the pressure areas formed at the nip junction of ink

rollers, dampening system rollers, and printing plates of the printing press. Whatever the mechanism might be, all successful lithographic inks when sampled from the inking system rollers are found to contain from about one percent to about as high as 40 percent of water, more or less, within and after a few revolutions to several hundred revolutions after start-up of the printing press. During operation of the press, some of the inking rollers must unavoidably encounter surfaces containing water, such as the printing plate, from which contact a more or less gradual build up of water in the ink takes place, proceeding back through the inking train, often all the way to the ink reservoir. Consequently, the presence of water in the ink during lithographic printing is a common expected occurrence.

In lithographic printing press inking roller train systems, it is typically advantageous to select materials such that every other roller of the inking train participating in the film splitting and ink transfer is made from relatively soft, rubber-like, elastically compressible materials such as natural rubber, polyurethanes, Buna N and the like, materials that are known to have a natural affinity for ink and a preference for ink over water in the lithographic ink/water environment. The remaining rollers are usually made of a comparatively harder metallic material or occasionally a comparatively harder plastic or thermoplastic material such as mineral-filled nylons or hard rubber. This combination of alternating hard or incompressible and soft or compressible rollers is a standard practice in the art of printing press manufacture. It is important to note, although it has not yet been explainable, that the only practical and suitable metallic material the printing industry has found for use as the hard roller surface in lithographic inking systems is copper. Consequently, in the art of lithography, all metallic rollers for the inking system that will be subjected to relatively high dampening water concentration, namely those nearest the dampening system components and those nearest the printing plate, must and do have copper surface. Copper had been found long ago to possess consistent preference for ink in the presence of dampening water, unless it is inadvertently adversely contaminated. Means for cleaning or resensitizing contaminated copper surfaces towards ink are well known. When any other practical hard metal surface such as iron, steel, chrome, or nickel is used in the place of copper, debonding of ink from the roller surface by dampening water may sooner or later occur, with its attendant severely adverse printed quality and process control problems.

It is known that the relative propensity for debonding of ink from a surface depends in part, at least, upon the amount of water in the ink. Lithographic press manufacturers, have found, for instance, that although ink can readily be debonded from hardened steel in the presence of modest to large amounts of water, small amounts of water in the ink, for example less than a few percent, generally may not cause debonding. Consequently, rollers near or at the incoming reservoir of fresh ink, that is near the beginning of typical multi-roller inking trains and therefore relatively far from the sources of water may be successfully used when manufactured from various hard, non-copper metals such as iron and its various appropriate steel alloys. The balance of the relatively hard rollers are commonly made using copper for the reasons stated earlier.

Although there has been speculation about the reasons for the advantageous properties of copper for use in inking rollers, it remains uncertain why copper tends to prefer ink over water. For the purpose of this disclosure, this property will be referred to as oleophilic meaning ink loving or oil loving and hydrophobic or water shedding. As indicated, certain of the rubber and plastic roller materials may be useful as the hard rollers in conventional, long train inkers. These, too, have the oleophilic/hydrophobic/oil/water preference property, though perhaps for different scientific reasons than with copper.

In the case of metallic or polymeric rubber or plastic rollers, whether soft or hard, this oleophilic/hydrophobic behavior can be more or less predicted by measuring the degree to which droplets of ink oil and of dampening water will spontaneously spread out on the surface of the metal or polymer rubber or plastic. The sessile drop technique as described in standard surface chemistry textbooks is suitable for measuring this quality. Generally, oleophilic/hydrophobic roller materials will have an ink oil (Flint Ink Co.) contact angle of nearly 0° and a distilled water contact angle of about 90° or higher and these values serve to define an oleophilic/hydrophobic material.

We have found, for instance, that the following rules are constructive in but not restrictive for selecting materials according to this principle:

|                         |                                                                                                          |
|-------------------------|----------------------------------------------------------------------------------------------------------|
| Best                    | Water contact angle 90° or higher.<br>Ink Oil contact angle 10° or lower and spreading.                  |
| Maybe Acceptable        | Water contact angle 80° or higher.<br>Ink Oil contact angle 10° or lower and spreading.                  |
| Probably Not Acceptable | Water contact angle less than about 80°.<br>Ink Oil contact angle greater than 10° and/or non-spreading. |

Another related test is to place a thin film of ink on the material being tested, then place a droplet of dampening solution on the ink film. The longer it takes and the lesser extent to which the water solution displaces or debonds the ink, the greater is that materials' oleophilic/hydrophobic property.

Materials that have this oleophilic/hydrophobic property as defined herein will in practice in a lithographic printing press configuration accept, retain and maintain lithographic ink on its surface in preference to water or dampening solution when both ink and water are presented to or forced onto that surface. And it is this oleophilic/hydrophobic property that allows rollers used in lithographic press inking roller trains to transport ink from an ink reservoir to the substrate being printed without loss of printed-ink density control due to debonding of the ink by water from one or more of the inking rollers.

#### REFERENCES TO THE PRIOR ART

Warner in U.S. Pat. No. 4,287,827 describes a novel inking roller that is manufactured to have bimetal surfaces, for instance chromium and copper, which different roller surfaces simultaneously carry dampening solution and ink respectively to the form rollers of a simplified inking system. The Warner technology specifies planarity of the roller surface which is a distinct

departure from the instant invention. In the Warner technology, the ink-loving copper areas will carry an ink quantity corresponding to the thickness of the ink film being conveyed to it by preceding rollers in the inking system. Thus the primary metering of the ink is done separately from the bimetallic-surfaced roller or through the use of a flooded nip between the bimetal roller and a coacting resiliently-covered inking roller. This contrasts completely with the instant technology, in which one utilizes a celled ink-loving roller which together with a doctor blade defines the amount of ink being conveyed to the form rollers and is therefore truly an ink-metering roller. In addition, the instant invention involves using an independent dampening system, rather than relying on hydrophilic land areas of the inking roller as in the Warner technology to supply dampening solution to the printing plate.

A number of celled or recessed or anilox-type ink metering rollers have been described in trade and technical literature. The American Newspaper Publishers Association (ANPA) has described in Mataila and Navi U.S. Pat. No. 4,407,196 a simplified inking system for letterpress printing, which uses chromium or hardened steel or hard ceramic materials like tungsten carbide and aluminum oxide as the metering roller material of construction. These hard materials are advantageously used to minimize roller wear in a celled ink-metering roller inking system operating with a continuously-scraping coextensive doctoring blade. Letterpress printing does not require purposeful and continuous addition of water to the printing system for image differentiation and therefore debonding of ink from these inherently hydrophilic rollers by water does not occur and continuous ink metering control is possible. Attempts have been made to adopt the ANPA system to lithographic printing without benefit of the instant technology. The ANPA technology rollers are naturally both oleophilic and hydrophilic and will sooner or later fail by water debonding ink from the metering roller. The failure will be particularly evident at high printing speeds where build-up of water occurs more rapidly and for combinations of printing formats and ink formulations that have high water demand. The instant technology avoids these sensitivities.

Granger in U.S. Pat. No. 3,587,463 discloses the use of a single celled inking roller, which operates in a mechanical sense, substantially like the inking system schematically illustrated in this disclosure as FIGS. 4 and 5, excepting that no provision for dampening, therefore for lithographic printing was disclosed nor anticipated. Granger's system will not function as the present invention for reasons similar to that already presented in the Mataila and Navi case.

#### SUMMARY OF THE INVENTION

This invention relates to method, materials and apparatus for metering ink in modern, high-speed lithographic printing press systems, wherein means are provided to simplify the inking system and to simplify the degree of operator control or attention required during operation of the printing press.

The amount of ink reaching the printing plate is controlled primarily by the dimensions of depressions or cells in the surface of a metering roller and by a coextensive scraping or doctor blade that continuously removes virtually all the ink from the celled metering roller except that carried in the cells or recesses.

The ink metering roller is composed of hardened steel of more-or-less uniform surface composition, engraved or otherwise manufactured to have accurately-dimensioned and positioned cells or recesses in said surface and lands or bearing regions which comprise all the roller surface excepting said cells, which cells and doctor blade serve to precisely meter a required volume of ink. To assure economically acceptable metering roller lifetimes, without serious deviation of the metering roller's ink control function, the metering roller is selected from materials having an outer-surface of Rockwell hardness at least about R<sub>c</sub>55 and is treated by a black-oxidizing process to have a permanent ink-accepting quality and a permanent water-rejecting quality.

A primary objective of this invention is to provide a simple, inexpensive manufacturing method and roller made therefrom that insures the economically practical operation of a simple system for continuously conveying ink to the printing plate in lithographic printing press systems.

Another primary objective of this invention is to provide a roller with a celled metering surface that continuously measures and transfers the correct, predetermined quantity of ink to the printing plate and thereby to the substrate being printed, without having to rely on difficult-to-control slip-nips formed by contact of smooth inking rollers driven at different surface speeds from one another.

Another object of this invention is to provide a metering roller surface that is sufficiently hard and wear-resistant to allow long celled-roller lifetimes despite the scraping, wearing action of a doctor blade substantially in contact with it.

Still another objective of this invention is to provide automatic uniform metering of precisely controlled amounts of ink across the press width without necessity for operator interference as for instance in the setting of inking keys common to the current art of lithographic printing.

A further objective is to advantageously control the amount of detrimental starvation ghosting typical of simplified inking systems by continuously overfilling precisely-formed recesses or cells in a metering roller surface with ink during each revolution of said roller, then immediately and continuously scraping away all of the ink picked up by said roller, excepting that retained in said cells or recesses, thereby presenting the same precisely-metered amounts of ink to the printing plate form rollers each and every revolution of the printing press system.

Yet another object of this invention is to provide material and method for assuring that aqueous lithographic dampening solutions and their admixtures with lithographic inks do not interfere with the capability of a celled ink-metering roller to continuously and repeatedly pick-up and transfer precise quantities of ink.

These and other objectives and characteristics of this invention will become apparent by referring to the following descriptions and drawings and disclosures.

#### DESCRIPTION OF DRAWINGS

Drawings of preferred and alternative embodiments of the invention are attached for better understanding of the elements discussed in this disclosure. These embodiments are presented for clarity and are not meant to be restrictive or limiting to the spirit or scope of the invention, as will become apparent in the body of the disclosure.

FIG. 1 is a schematic end elevation of one preferred application of the inking roll of this invention;

FIG. 2 is a perspective view of the combined elements of FIG. 1;

FIG. 3 is a schematic showing a cell pattern which may be used in this invention;

FIG. 4 is an alternative cell pattern;

FIG. 5 is another cell pattern that can be advantageously used with this invention;

FIG. 6 is a cross-sectional view through a portion of an ink metering roll showing the relative dimensions between lands and valleys;

FIG. 7 is a view similar to FIG. 6 illustrating different dimensioning;

FIG. 8 is a schematic cross-sectional view of a portion of a roll surface as it would be after nitriding and oxidizing; and

FIG. 9 is a photomicrograph having the microporosity of a roll that has been nitrided and oxidized.

#### DESCRIPTION OF THE PREFERRED EMBODIMENT

Referring to FIGS. 1 and 2, an inker configuration suited to the practice of this invention in offset lithography consists of an ink-reservoir or ink-fountain 10 and/or a driven ink-fountain roller 11, a press-driven oleophilic/hydrophobic engraved or cellular roller 12, a reverse-angle metering blade or doctor-blade 13, and friction driven form rollers 14 and 15, which supply ink to a printing plate 16 mounted on plate-cylinder 20 and this in turn supplies ink to for example a paper web 21 being fed through the printing nip formed by the blanket cylinder 25 and the impression cylinder 26. All of the rollers in FIGS. 1 and 2 are configured substantially parallel axially.

The celled metering roller 12 of FIGS. 1, 2, 3, 4 and 5 is the novel element of this invention. It consists of engraved or otherwise-formed, patterned cells or depressions in the surface, the volume and frequency of the depressions being selected based on the volume of ink needed to meet required printed optical density specifications. The nature of this special roller is made clear elsewhere in this disclosure and in particular in FIGS. 3, 4 and 5 which depict suitable alternative patterns and cross-sections. Generally the celled metering roller will be driven at the same speed as the printing cylinders, typically from about 500 to 2000 revolutions per minute.

The doctor blade 13 depicted schematically in FIG. 1 and in perspective in FIG. 2 is typically made of flexible spring steel about 6 to 10 mils thick, with a chamfered edge to better facilitate precise ink removal. Mounting of the blade relative to the special metering roller is critical to successful practice of this invention but does not constitute a claim herein since doctor blade mounting techniques suitable for the practice of this invention are well known. A typical arrangement for setting the doctor blade is illustrated in FIGS. 1 and 2. The doctor blade or the celled metering roller may be vibrated axially during operation to distribute the wear patterns and achieve additional ink film uniformity.

Typically, differently-diamented form-rollers 14 and 15 of FIG. 1 are preferred in inking systems to help reduce ghosting in the printed images. These rollers will generally be a resiliently-covered composite of some kind, typically having a Shore A hardness value between about 22 and 28. The form rollers preferably are mutually independently adjustable to the printing plate

cylinder 20 and to the special metering roller 12 of this invention, and pivotally mounted about the metering roller and fitted with manual or automatic trip-off mechanisms as is well known in the art of printing press design. The form rollers are typically and advantageously friction driven by the plate cylinder 20 and/or the metering roller 12.

We have found that hard, wear-resistant materials available for manufacture of an inking roller are naturally hydrophilic, rather than hydrophobic. And the commonly-used hard metals such as chromium or nickel and hardened iron alloys such as various grades of steel, as well as readily-available ceramic materials such as aluminum oxide and tungsten carbide prefer to have a layer of water rather than a layer of ink on their surfaces when both liquids are present. This preference is enhanced in situations where portions of the fresh material surfaces are continuously being exposed because of the gradual wearing action of a doctor blade. It is also enhanced if that fresh, chemically-reactive metal surface tends to form hydrophilic oxides in the presence of atmospheric oxygen and water from the lithographic dampening solution. Oxidizing corrosion to form iron oxide  $Fe_2O_3$  in the case of steel compounds is a typical example. Thus, although various grades of steel, chromium and its oxides, nickel and its oxides will readily operate as the uppermost surface in an ink-metering roller for printing systems not requiring water, such as letterpress printing, these same surfaces will become debonded of ink when sufficient dampening water penetrates to the roller surface, as for instance, in the practice of lithographic printing. The action of a doctor blade on a rotating ink-metering roller more-or-less rapidly exposes fresh metering roller surface material which prefers water. This is more readily understood if one considers that hydrophilic, water-loving, surfaces are also oleophilic, oil-loving in the absence of water, such as when fresh, unused, water-free lithographic ink is applied to a steel or ceramic roller. Initially the ink exhibits good adhesion and wetting to the roller. During printing operations, as the water content in the ink increases, a point will be reached when a combination of roller nip pressures and increasing water content in the ink force water through the ink layer to the roller surface thereby debonding the ink from these naturally hydrophilic surfaces, the ink layer thereby becoming more-or-less permanently replaced by the more stable water layer.

We have discovered that by treating a nitride-hardened steel roller in a manner that it is oxidized to the so-called black form of iron oxide,  $Fe_3O_4$ , we can completely avoid the ink debonding action that we have just described. While not completely understood, it appears that the  $Fe_3O_4$  layer or coating passivates the steel surface against corrosive oxidation, which corrosion otherwise occurs readily and naturally, resulting in the formation of the fully-oxidized, hydrophilic iron oxide,  $Fe_2O_3$ , on the steel roller surfaces. Additionally and surprisingly, the method of our invention imparts excellent, permanent oleophilic/hydrophobic character to the steel roller surface. By this simple means we have discovered a unique method for imparting to a hardened steel roller both a preference of its surface for ink or oil rather than water and for imparting the resistance to corrosion or chemical change necessary to retain this oil-loving or ink-loving property during extended lithographic printing operations.

In the practice of our invention, we may for instance gas-nitride-harden or liquid-nitride-harden an engraved steel roller to a minimum case depth of about three mils or more, then dip the roller one or more times into a hot 300° to 450° F. oil bath containing oxidizing chemicals appropriate to formation on the surface of the roller what is termed in the trade black oxide.

Nitriding to harden the steel roller for our invention is particularly suitable as it allows forming the ink-carrying cells by simple well-known means such as mechanical engraving of a nitriding steel grade, such as AISI 4140 or 5640, prior to hardening. The nitride hardening step is a relative low-temperature, non-quenching process that avoids distortion accompanying most heat-hardening treatments.

Although we believe  $Fe_3O_4$  to be a primary chemical species on the roller surface of this invention, we recognize that the presence of for instance iron nitrides in the hardened roller surface, before being oxidized, may result in the formation of various combinations of iron, nitrogen, and/or carbon oxides at the surface of the steel when the roller is subsequently oxidized.

In a specific instance, a 4.42 inch diameter, 36 inch face roller of AISI 4150 steel was machine engraved to have standard 250 TPB truncated bipyramid cells, substantially as illustrated in FIG. 6. The roller was gas-nitride hardened by subjecting it to dissociated  $N_2/NH_3$  vapors at high temperature according to a proprietary process owned by J & A Heat Treating Company, Schaumberg, Ill. to a calculated Rockwell C scale hardness of about 60. The roller was then subjected to a proprietary black oxidizing process by Western Rustproof Company of Chicago, Ill., which consisted of two treatments of 5 to 10 minutes each in a heated chemical oil bath, followed by air cooling. The roller was fitted to a simplified lithographic inker system substantially as illustrated in FIGS. 1 and 2 and run for 1.5 million impressions (750,000 revolutions) with no significant loss in print quality or in ink metering capability.

In a second illustration a roller was made in the same manner as that set forth in example 1 above, except that the cells were machine engraved according to the pattern of FIG. 7 and the gas nitride hardening was done by Lindberg Corporation of Chicago, Ill. to the same specifications as the example above, according to their proprietary technology. After demonstrating failure as a long run lithographic ink metering roller on the press of example 1, the roller was black-oxide treated as in example 1. Subsequent printing tests using the same press configuration resulted in more than five million revolutions with no visible loss in print quality or in ink metering capability.

A metering roller made substantially as indicated in the first illustration but using AISI 1018 steel, a non-nitride-hardening grade, exhibited good hydrophobic/oleophilic surface properties when first used on press. Within one-half million to two million revolutions the roller was worn beyond acceptability as evidenced by severe loss of printed optical density.

Also the surface chemical properties had adversely changed from hydrophobic/oleophilic to hydrophilic/oleophilic.

Tests run on the black-oxide steel roller that had been liquid nitrided to a calculated 12 mil case depth and then double dipped, black-oxide treated revealed that the composition of the black-oxide had an atomic oxygen to iron ratio of 1.2 to 1.3 at the surface, which is consistent

with the composition of magnetite ( $Fe_3O_4$ ) which would give a ratio of 1.33. At approximately 1100 Å (Angstroms) depth, the composition was less than one oxygen per atom iron. Virtually no nitride was apparent to a depth of about 1100 Angstroms. Consequently the magnetite is oxygen-starved, that is, in a chemically-reduced condition. The reduced iron oxides are expected to be more basic as compared with the more acidic fully-oxidized iron oxides typically present in thin passive films formed on untreated steel exposed to air. This basic property of the iron oxide formed by the black oxide treatment of nitrided steel may relate to its apparent oleophilic/hydrophobic behavior.

Schematically, FIG. 8 shows the microporous structure 30 that was formed on the surface of roll 31 which was comprised of two to three millimicron crystallites of the oxide. FIG. 9 shows the actual microporosity of the nitrided and oxidized surface. There did appear to be some smoothing and smearing of these crystallites in the region where the sample was purposely worn. However, the surface compositions in the worn and as received region showed very little change from that just described.

Although the present invention has been described in connection with preferred embodiments, it is to be understood that modifications and variations may be resorted to without departing from the spirit and scope of the invention as those skilled in the art will readily understand. Such modifications and variations are considered to be within the purview and scope of the invention and the appended claims.

What is claimed is:

1. An ink metering roller for use in lithographic printing comprising:
  - a. an engraved base roller of suitable diameter and length, selected from nitride-hardenable steel;
  - b. an outer zone of not less than about 3 mils thickness that is nitride-hardened to an  $R_c$  value of not less than about 55;

- c. an outermost microporous iron oxide layer on said outer surface of said steel roller that consists essentially of  $Fe_3O_4$ .
2. An ink metering roller as defined in claim 1 wherein the oxygen to iron ratio of the metal oxide is less than the stoichiometric ratio of 1.33 for  $Fe_3O_4$ .
3. An ink metering roller as defined in claim 2 wherein the atomic oxygen to iron ratio of the metal oxide on the surface of said roll ranges from about 1.2 to 1.3.
4. An ink metering roller as defined in claim 3 wherein the atomic oxygen to iron ratio decreases in the direction inwardly from the surface of said roller.
5. A process for producing an ink metering roller for use in lithographic printing comprising the steps of:
  - a. providing a nitride-hardenable steel roll of preselected diameter and surface configuration;
  - b. nitriding the roll to a preselected depth to produce a face case of increased hardness and;
  - c. oxidizing the nitrided surface of the roll to produce a microporous layer or iron oxide whose composition consists principally of the oxide  $Fe_3O_4$ .
6. The process as defined in claim 5 wherein said oxidizing treatment is effected by immersing the roll 25 into an oxidizing oil bath at a temperature of from about 300° to 450° F.
7. The process as defined in claim 5 wherein said roll is nitrided for a time to form a case of not less than about 3 mils thickness and not less than about  $R_c 55$  hardness.
8. An inking system for use in lithographic printing consisting at least in part of a nitride-hardenable steel ink metering roller coextensive with the width of a lithographic printing press system, said metering roller consisting of recesses or cells of appropriate frequency and 30 volume to deliver a uniform and acceptable ink density by means of auxiliary rollers to a substrate being printed by said printing press system, and consisting of land areas between said cells or recesses upon which rests during operation a reverse-angle ink-doctoring blade coextensive with said ink-metering roller, said roller having surfaces that are made oleophilic and hydrophobic by black-oxide treatment of said roller surface.

\* \* \* \* \*